

(No Model.)

S. R. & A. C. BRADLEY.  
PROCESS OF MANUFACTURING OXIDES.

No. 404,254.

Patented May 28, 1889.



Witnesses.

Walter Stalter  
Jas. S. Stamer

Inventors  
S. R. Bradley  
A. C. Bradley  
By their Attorney

J. S. Remick

# UNITED STATES PATENT OFFICE.

STEPHEN ROWE BRADLEY AND ARTHUR CROSSMAN BRADLEY, OF BROOKLYN, NEW YORK.

## PROCESS OF MANUFACTURING OXIDES.

SPECIFICATION forming part of Letters Patent No. 404,254, dated May 28, 1889.

Application filed February 18, 1888. Serial No. 264,516. (No specimens.)

*To all whom it may concern:*

Be it known that we, STEPHEN ROWE BRADLEY and ARTHUR CROSSMAN BRADLEY, both of Brooklyn, in the county of Kings and State of New York, have made an invention of certain new and useful Improvements in the Process of Manufacturing Oxides of Easily-Oxidizable Metals, such as Litharge and the Oxide of Zinc; and we do hereby declare that the following, in connection with the accompanying drawings, is a full, clear, and exact description and specification of the same.

The object of our invention is to enable the metal to be oxidized rapidly and at a small cost; and the invention consists of an improved process by which the object is accomplished.

The several parts of the invention are set forth in detail in the claims at the close of this specification. In order that they may be fully understood, we have represented in the accompanying drawings, and will proceed to describe, the form of apparatus which we prefer to use for the purpose, and will describe the mode of operation by its use.

Figure 1 of said drawings represents a longitudinal section of said apparatus, and Fig. 2 represents a larger face view of the form of gas-nozzle which we prefer to use. Fig. 3 represents a modified form of combined gas-injector and comminutor.

One of the principal members of the apparatus represented in said drawings is the oxidizing-chamber A, which may be ten feet long, three feet broad, and six feet in height. At one end of this chamber is the combined gas-injector and comminutor. This consists of a gas-nozzle, B, and a feeder, C, for delivering a stream of molten metal to the current of gas proceeding from the gas-nozzle. The orifice of the gas-nozzle is made preferably of crescent form, (as represented in front view at Fig. 2,) and the supply of gas to this nozzle is controlled by a valve, d, in the supply pipe. The feeder C consists of a funnel, e, terminating in a feed-pipe, f, which delivers the molten metal directly to the jet or blast of gas proceeding from the gas-nozzle, and the delivery of the metal is controlled by a movable gate or valve, g, which is fitted to the feed-pipe f.

The combined gas-injector and comminutor is preferably arranged in a case, H, which is secured to one of the end walls of the oxidizing-chamber outside of an opening, I, provided for the purpose, the gas-injector being arranged in an air-pipe, J, in which the injector-nozzle is preferably adjustable, so that it may be set by trial at the most advantageous position for operation.

The end of the oxidizing-chamber which is farthest from the gas-injector and comminutor is connected with a dust-collector. The construction of dust-collector which we prefer to employ is a bag collector such as is used in the manufacture of oxide of zinc, and its pipes may be connected with the oxidizing-chamber by a connecting-pipe, L, of sheet-iron. The pipes and number of bags m may be extended as found necessary to collect the dust oxide which passes from the chamber A and permit the gaseous products to escape through the cloth of the bags, leaving the dust in the bags.

In operating with the above-described apparatus inflammable gas (such, for example, as natural gas) is supplied to the gas-injector B at the requisite pressure, the pressure which we recommend for the purpose being eighty pounds per square inch. The gas is turned on and is lighted, (through an aperture in the side of the casing H, provided for that purpose.) Then molten metal (lead, for example) is fed in a stream to the jet or blast of gas by means of the feeder C. The molten metal is thus subjected to the action of a blast of inflammable gas under pressure, and the action of the jet or blast upon the stream of molten metal comminutes it by separating it into minute globules and distributes it in the atmosphere of the oxidizing-chamber, while at the same time the gas, being in a burning condition, furnishes the heat required to cause the metal to burn in the air in the oxidizing-chamber, a supply of air being carried through the air-tube J by the action of the blast, so that when the air-tube is open the metal is subjected to a combined blast of burning gas and air. The metal is thus simultaneously comminuted, distributed in the oxidizing-chamber, and heated to the burning temperature by the jet of gas proceeding

from the injector. The comminuted metal burns rapidly and is converted into its oxide. The chamber forms an inclosed space in which the distributed metal and the oxide produced are under confinement, so that the loss that would accrue if the burning was effected in the open air is prevented. Such of the oxide as falls in the oxidizing-chamber collects therein and may be removed at intervals through doorways *a*, provided for the purpose, these doorways being closed by doors when the operation is proceeding. Such oxide as does not drop in the oxidizing-chamber is carried with the current of the gaseous products of combustion and any excess of air into the dust-collector and is collected therein.

If the oxidizing-chamber is made large enough, a supplementary dust-collector is not necessary, as the oxidizing-chamber in such case operates both as oxidizing-chamber and dust-collector, and the collection in a long oxidizing-chamber may be facilitated by the use of partitions arranged as is well understood, so as to make the current of mixed gaseous products and oxide take a zigzag course.

In the mode of practicing our invention thus far described the inflammable gas is supplied centrally of the compound gas-injector and comminutor, and the air is supplied laterally of the gas; but this arrangement of the supplies may be reversed and the air may be supplied under high pressure. In practicing our invention with this variation we prefer to construct the compound gas-injector and comminutor as represented in section at Fig. 3. In this case the central nozzle, *B*, may be supplied with air under pressure, (a pressure of eighty pounds per square inch being a good pressure for the purpose,) while the inflammable gas may be supplied through lateral pipes or through a pipe, *J*, which surrounds the central nozzle, and may then be supplied

at a comparatively low pressure, as the force of the air under the high pressure will be sufficient to comminute and distribute the molten metal, while the inflammable gas, which mixes with the air and is burned, supplies the requisite heat for oxidation. The chamber *A* and the dust-collector used with this variation of the process may be the same as previously described.

The apparatus above described is not herein claimed, as we have made the same the subject of a separate application for a patent, which application is numbered 260,384.

We claim as our invention—

1. The process, substantially as before set forth, of manufacturing metallic oxides by subjecting molten metal in a stream to a blast under confinement in the presence of burning inflammable gas.

2. The process, substantially as before set forth, of simultaneously comminuting molten metal, distributing it, and oxidizing it, which consists in subjecting the molten metal in a stream to a blast and burning inflammable gas in a confined space, whereby waste is prevented.

3. The process, substantially as before set forth, of simultaneously comminuting molten metal, distributing it, heating it to a burning-point, and saving the oxide, which consists in subjecting the molten metal in a stream and under confinement to a blast and burning inflammable gas and collecting the oxide produced.

In witness whereof we have hereunto set our hands this 10th day of February, A. D. 1888.

STEPHEN ROWE BRADLEY.  
ARTHUR CROSSMAN BRADLEY.

Witnesses:

JOHN B. FROTHINGHAM,  
FREDK. J. SHARP.